



US008133136B2

(12) **United States Patent**  
**Umezawa et al.**

(10) **Patent No.:** **US 8,133,136 B2**  
(b4) **Date of Patent:** **Mar. 13, 2012**

(54) **MULTI-PIECE SOLID GOLF BALL**

(75) Inventors: **Junji Umezawa**, Chichibu (JP); **Hiroshi Higuchi**, Chichibu (JP); **Daisuke Arai**, Chichibu (JP); **Hiroyuki Nagasawa**, Chichibu (JP)

(73) Assignee: **Bridgestone Sports Co., Ltd.**, Tokyo (JP)

(\*) Notice: Subject to any disclaimer, the term of this patent is extended or adjusted under 35 U.S.C. 154(b) by 274 days.

(21) Appl. No.: **12/361,045**

(22) Filed: **Jan. 28, 2009**

(65) **Prior Publication Data**

US 2010/0190575 A1 Jul. 29, 2010

(51) **Int. Cl.**

**A63B 37/06** (2006.01)

(52) **U.S. Cl.** ..... **473/374**

(58) **Field of Classification Search** ..... **473/373, 473/374**

See application file for complete search history.

(56) **References Cited**

## U.S. PATENT DOCUMENTS

|               |         |                                     |
|---------------|---------|-------------------------------------|
| 5,306,760 A   | 4/1994  | Sullivan                            |
| 5,312,857 A   | 5/1994  | Sullivan                            |
| 5,830,085 A   | 11/1998 | Higuchi et al.                      |
| 6,129,640 A * | 10/2000 | Higuchi et al. ..... <b>473/374</b> |
| 6,277,035 B1  | 8/2001  | Sullivan et al.                     |
| 6,277,924 B1  | 8/2001  | Hamada et al.                       |
| 6,409,614 B1  | 6/2002  | Binette et al.                      |
| 6,561,928 B2  | 5/2003  | Binette et al.                      |
| 6,642,314 B2  | 11/2003 | Sone et al.                         |
| 6,663,507 B1  | 12/2003 | Watanabe et al.                     |
| 6,991,562 B2  | 1/2006  | Sullivan et al.                     |

|                   |         |                                       |
|-------------------|---------|---------------------------------------|
| 7,160,211 B2      | 1/2007  | Sullivan et al.                       |
| 7,294,680 B2      | 11/2007 | Sone et al.                           |
| 2005/0239578 A1 * | 10/2005 | Watanabe et al. ..... <b>473/371</b>  |
| 2006/0116221 A1 * | 6/2006  | Watanabe et al. ..... <b>473/371</b>  |
| 2007/0197313 A1 * | 8/2007  | Watanabe et al. ..... <b>473/371</b>  |
| 2009/0209366 A1 * | 8/2009  | Kashihama et al. ..... <b>473/373</b> |

## FOREIGN PATENT DOCUMENTS

|    |               |         |
|----|---------------|---------|
| JP | 7-268132 A    | 10/1995 |
| JP | 11-35633 A    | 2/1999  |
| JP | 2002-293996 A | 10/2002 |
| JP | 2004-49913 A  | 2/2004  |
| JP | 3505922 B2    | 3/2004  |
| WO | 98/46671 A1   | 10/1998 |

\* cited by examiner

Primary Examiner — Raeann Gorden

(74) Attorney, Agent, or Firm — Sughrue Mion, PLLC

(57) **ABSTRACT**

The invention provides a multi-piece solid golf ball composed of a solid core, a cover, at least one intermediate layer interposed therebetween, and a plurality of dimples on a surface of the ball. The respective initial velocities (m/s) of the core, a sphere I composed of the core encased by the intermediate layer, and the golf ball satisfy formula A below, and the respective deflections (mm) of the core, the sphere I composed of the core encased by the intermediate layer, and the golf ball, when compressed under a final load of 130 kg from an initial load of 10 kgf, satisfy formula B below:

$$\begin{aligned} & \text{(initial velocity of core - initial velocity of sphere I)}^2 + \\ & \text{(initial velocity of sphere I - initial velocity of golf ball)}^{2 \leq 0.40} ; \end{aligned} \quad \text{Formula A:}$$

$$0.30 < \text{(deflection of core - deflection of sphere I)}^2 + \\ \text{(deflection of sphere I - deflection of golf ball)}^{2 < 0.70} . \quad \text{Formula B:}$$

The golf ball of the invention has a good feel, an excellent spin performance on approach shots and an excellent distance, in addition to which it has an excellent scuff resistance and durability.

**3 Claims, 1 Drawing Sheet**



**FIG.1****FIG.2**

## 1

## MULTI-PIECE SOLID GOLF BALL

## BACKGROUND OF THE INVENTION

The present invention relates to a multi-piece solid golf ball of three or more layers which is composed of a solid core, an intermediate layer and a cover, and is endowed with excellent properties such as flight performance, feel on impact, controllability, and scuff resistance.

In recent years, the number of layers in solid golf balls has been increased from the conventional two-piece ball construction composed of a solid core and a cover by additionally providing an intermediate layer between the solid core and the cover, and efforts are being made to optimize each of the layers. Various three-piece golf balls have been disclosed in which a good flight performance and an excellent durability, feel and controllability are achieved by giving the core itself an optimized hardness profile and by providing the ball as a whole—including the core, the intermediate layer and the cover—with an optimized hardness profile.

For example, JP No. 3505922 (and the corresponding specification of U.S. Pat. No. 5,830,085) discloses a three-piece solid golf ball having a core, an intermediate layer and a cover, which ball satisfies the following relationship: core center hardness<core surface hardness<intermediate layer hardness<cover hardness. However, this golf ball has a low rebound.

JP-A 2004-49913 (and the corresponding specification of U.S. Pat. No. 6,663,507) discloses a multi-piece solid golf ball which has, between a core and a cover, an intermediate layer composed primarily of a binary copolymer and having a Shore D hardness of at least 50. However, the flight performance and scuff resistance of this golf ball leave something to be desired.

U.S. Pat. Nos. 6,409,614, 6,277,035, 6,991,562 and 7,160,211 disclose multi-piece solid golf balls having a core, a soft inner cover and a hard outer cover, which outer cover is a cover having a high Shore D hardness. However, these golf balls do not have both a satisfactory controllability and a satisfactory feel. Hence, there has remained room for improvement.

In the golf ball of U.S. Pat. No. 6,561,928, the total thickness of the cover encasing the core is too large, resulting in a decrease in flight performance.

Because the many multi-piece solid golf balls which have been disclosed to date fail to satisfy all the desired attributes—namely, flight performance, feel on impact, controllability/spin performance, scuff resistance and durability, a need has been felt for further improvement.

## SUMMARY OF THE INVENTION

It is therefore an object of the present invention to provide a multi-piece golf ball of at least three layers which has a solid core, an intermediate layer and a cover, and which is endowed with an excellent feel on impact, controllability, flight performance and scuff resistance.

The inventors have conducted extensive investigations in order to achieve the above object. As a result, they have discovered that, in a multi-piece solid golf ball having a core, an intermediate layer and a cover, by minimizing the differences in initial velocity between the respective layers and optimizing the differences in deflection under specific loading between the respective layers, the ball can be imparted with a good feel on impact and an excellent spin performance on approach shots, in addition to which a lower spin rate can be achieved on full shots, improving the distance of the ball.

## 2

Accordingly, the invention provides the following multi-piece solid golf balls.

[1] A multi-piece solid golf ball comprising a solid core, a cover, at least one intermediate layer interposed therebetween, and a plurality of dimples on a surface of the ball, wherein the respective initial velocities (m/s) of the core, a sphere I composed of the core encased by the intermediate layer, and the golf ball, as measured by a method set forth in the Rules of Golf using an initial velocity measuring apparatus of the same type as a USGA drum rotation-type initial velocity instrument, satisfy formula A below, and the respective deflections (mm) of the core, the sphere I composed of the core encased by the intermediate layer, and the golf ball, when compressed under a final load of 130 kgf from an initial load of 10 kgf, satisfy formula B below:

$$(initial\ velocity\ of\ core - initial\ velocity\ of\ sphere\ I)^2 + (initial\ velocity\ of\ sphere\ I - initial\ velocity\ of\ golf\ ball)^2 < 0.40; \quad \text{Formula A}$$

$$0.30 < (deflection\ of\ core - deflection\ of\ sphere\ I)^2 + (deflection\ of\ sphere\ I - deflection\ of\ golf\ ball)^2 < 0.70. \quad \text{Formula B}$$

[2] The multi-piece solid golf ball of [1], wherein the cover has a material hardness that is higher than a material hardness of the intermediate layer, and which satisfies formula C below:

$$0 < [material\ hardness\ (Shore\ D)\ of\ intermediate\ layer \times intermediate\ layer\ thickness\ (mm)] - [material\ hardness\ (Shore\ D)\ of\ cover \times cover\ thickness\ (mm)] < 40. \quad \text{Formula C}$$

[3] The multi-piece solid golf ball of [1] which satisfies formula D below:

$$1.2 < intermediate\ layer\ thickness / cover\ thickness < 1.7. \quad \text{Formula D}$$

[4] The multi-piece solid golf ball of [1], wherein the intermediate layer is composed primarily of a material obtained by mixing under applied heat:

100 parts by weight of a resin component of

- (a) from 95 to 50 wt % of an olefin-unsaturated carboxylic acid-unsaturated carboxylic acid ester random terpolymer and/or a metal salt thereof,
- (b) from 0 to 10 wt % of an olefin-unsaturated carboxylic acid random copolymer and/or a metal salt thereof, and
- (c) from 5 to 50 wt % of a thermoplastic block copolymer having a crystalline polyolefin block and a polyethylene/butylene random copolymer, with

(d) from 5 to 100 parts by weight of a fatty acid or fatty acid derivative having a molecular weight of from 280 to 1500, and

(e) from 0.1 to 10 parts by weight of a basic inorganic metal compound capable of neutralizing acid groups within components (a), (b) and (d);

and the intermediate layer has a Shore D hardness difference with a surface of the solid core of within  $\pm 10$ .

[5] The multi-piece solid golf ball of [1], wherein the intermediate layer is composed primarily of a material obtained by mixing under applied heat:

100 parts by weight of a resin component of

- (a) from 0 to 20 wt % of an olefin-unsaturated carboxylic acid-unsaturated carboxylic acid ester random terpolymer and/or a metal salt thereof,
- (b) from 95 to 50 wt % of an olefin-unsaturated carboxylic acid random copolymer and/or a metal salt thereof, and
- (c) from 5 to 50 wt % of a thermoplastic block copolymer having a crystalline polyolefin block and a polyethylene/butylene random copolymer, with

(d) from 5 to 100 parts by weight of a fatty acid or fatty acid derivative having a molecular weight of from 280 to 1500, and

(e) from 0.1 to 10 parts by weight of a basic inorganic metal compound capable of neutralizing acid groups within components (a), (b) and (d);

and the intermediate layer has a Shore D hardness difference with a surface of the solid core of within  $\pm 10$ .

#### BRIEF DESCRIPTION OF THE DIAGRAMS

FIG. 1 is a cross-sectional view showing a multi-piece solid golf ball according to one embodiment of the invention.

FIG. 2 is a plan view of the surface of the golf balls in the examples (Dimple I).

#### DETAILED DESCRIPTION OF THE INVENTION

Describing the invention more fully below in conjunction with the attached diagrams, the multi-piece golf ball of the invention has at least a three-piece construction composed of a solid core 1, an intermediate layer 2 encasing the solid core 1, and a cover 3 encasing the intermediate layer 2. A plurality of dimples D are formed on the surface of the cover 3. FIG. 1 shows a construction in which the solid core 1, the intermediate layer 2, and the cover 3 are composed of one layer each, although these may have multilayer constructions of two or more layers. If necessary, the solid core 1, the intermediate layer 2 and the cover 3 may each have a multilayer construction. When the solid core, intermediate layer or cover described below has a multilayer construction, the multiple layers together should be configured in such a way as to collectively satisfy the conditions which pertain to that piece of the golf ball.

First, the solid core is described. The solid core is molded under the application of heat from a rubber composition containing polybutadiene as the base rubber.

Here, the polybutadiene has a cis-1,4 bond content of at least 60%, preferably at least 80%, more preferably at least 90%, and most preferably at least 95%.

It is recommended that the polybutadiene have a Mooney viscosity ( $ML_{1+4}(100^\circ C.)$ ) of at least 30, preferably at least 35, more preferably at least 40, and even more preferably at least 50, but not more than 100, preferably not more than 80, more preferably not more than 70, and most preferably not more than 60.

The term "Mooney viscosity" used herein refers to an industrial indicator of viscosity as measured with a Mooney viscometer, which is a type of rotary plastometer (JIS-K6300). The unit symbol used is  $ML_{1+4}(100^\circ C.)$ , where "M" stands for Mooney viscosity, "L" stands for large rotor (L-type), "1+4" denotes a pre-heating time of 1 minute and a rotor rotation time of 4 minutes, and "100°C." indicates that measurement was carried out at a temperature of  $100^\circ C$ .

The molecular weight distribution  $M_w/M_n$  (where  $M_w$  stands for the weight-average molecular weight, and  $M_n$  stands for the number-average molecular weight) of the above polybutadiene is at least 2.0, preferably at least 2.2, more preferably at least 2.4, and even more preferably at least 2.6, but not more than 6.0, preferably not more than 5.0, more preferably not more than 4.0, and even more preferably not more than 3.4. If  $M_w/M_n$  is too small, the workability may worsen. On the other hand, if it is too large, the rebound may decrease.

The polybutadiene may be synthesized using a nickel or cobalt catalyst, or may be synthesized using a rare-earth

catalyst. Synthesis with a rare-earth catalyst is especially preferred. A known rare-earth catalyst may be used for this purpose.

Examples include catalysts obtained by combining a lanthanum series rare-earth compound, an organoaluminum compound, an alumoxane, a halogen-bearing compound and, if necessary, a Lewis base.

In the present invention, the use of a neodymium catalyst containing a neodymium compound as the lanthanum series rare-earth compound is advantageous because it enables a polybutadiene rubber having a high 1,4-cis bond content and a low 1,2-vinyl bond content to be obtained at an excellent polymerization activity. Preferred examples of such rare-earth catalysts include those mentioned in JP-A 11-35633.

When butadiene is polymerized in the presence of a rare-earth catalyst, bulk polymerization or vapor-phase polymerization may be carried out, with or without the use of a solvent. The polymerization temperature may be set to generally between  $-30^\circ C.$  and  $150^\circ C.$ , and preferably between 10 and  $100^\circ C.$

Alternatively, the polybutadiene may be obtained by polymerization using the rare-earth catalyst, followed by the reaction of an active end on the polymer with a terminal modifier.

Examples of terminal modifiers and methods for carrying out such a reaction includes those described in, for example, JP-A 11-35633, JP-A 7-268132 and JP-A 2002-293996.

The polybutadiene should be included in the rubber base in an amount of at least 60 wt %, preferably at least 70 wt %, more preferably at least 80 wt %, and most preferably at least 90 wt %. The upper limit in the amount of polybutadiene included is 100 wt % or less, preferably 98 wt % or less, and more preferably 95 wt % or less. When too little polybutadiene is included in the rubber base, it is difficult to obtain a golf ball having a good rebound.

Rubbers other than the above-described polybutadiene may be included and used together with the polybutadiene insofar as the objects of the invention are attainable. Illustrative examples include polybutadiene rubbers (BR), styrene-butadiene rubbers (SBR), natural rubbers, polyisoprene rubbers, and ethylene-propylene-diene rubbers (EPDM). These may be used singly or as combinations of two or more thereof.

The hot-molded solid core is formed using a rubber composition prepared by blending, as essential ingredients, specific amounts of an unsaturated carboxylic acid or a metal salt thereof, an organosulfur compound, an inorganic filler and an antioxidant with 100 parts by weight of the above-described base rubber.

The unsaturated carboxylic acid is exemplified by acrylic acid, methacrylic acid, maleic acid and fumaric acid. Acrylic acid and methacrylic acid are especially preferred.

Metal salts of unsaturated carboxylic acids that may be used include the zinc and magnesium salts of unsaturated fatty acids, such as zinc methacrylate and zinc acrylate. The use of zinc acrylate is especially preferred.

The amount of unsaturated carboxylic acid and/or metal salt thereof included per 100 parts by weight of the base rubber is preferably at least 20 parts by weight, more preferably at least 22 parts by weight, even more preferably at least 24 parts by weight, and most preferably at least 26 parts by weight, but preferably not more than 45 parts by weight, more preferably not more than 40 parts by weight, even more preferably not more than 35 parts by weight, and most preferably not more than 30 parts by weight. Including too much will result in excessive hardness, giving the ball an unpleasant feel when played. On the other hand, including too little will result in a decrease in the rebound.

An organosulfur compound may optionally be included. The organosulfur compound can be advantageously used to impart an excellent rebound. Thiophenols, thionaphthols, halogenated thiophenols, and metal salts thereof are recommended for this purpose. Illustrative examples include pentachlorothiophenol, pentafluorothiophenol, pentabromo-thiophenol, p-chlorothiophenol, and the zinc salt of pentachlorothiophenol; and diphenylpolysulfides, dibenzylpolysulfides, dibenzoylpolyisulfides, dibenzothiazoylpolyisulfides and dithiobenzoylpolyisulfides having 2 to 4 sulfurs. Diphenyldisulfide and the zinc salt of pentachlorothiophenol are especially preferred.

The amount of the organosulfur compound included per 100 parts by weight of the base rubber is preferably at least 0 part by weight, more preferably at least 0.1 part by weight, even more preferably at least 0.2 part by weight, and most preferably at least 0.4 part by weight, but preferably not more than 5 parts by weight, more preferably not more than 4 parts by weight, even more preferably not more than 3 parts by weight, and most preferably not more than 2 parts by weight. Including too much organosulfur compound may excessively lower the hardness, whereas including too little is unlikely to improve the rebound.

The inorganic filler is exemplified by zinc oxide, barium sulfate and calcium carbonate. The amount of the inorganic filler included per 100 parts by weight of the base rubber is preferably at least 5 parts by weight, more preferably at least 6 parts by weight, even more preferably at least 7 parts by weight, and most preferably at least 8 parts by weight, but preferably not more than 80 parts by weight, more preferably not more than 60 parts by weight, even more preferably not more than 40 parts by weight, and most preferably not more than 20 parts by weight. Too much or too little inorganic filler may make it impossible to achieve a suitable weight and a good rebound.

The organic peroxide may be a commercial product, examples of which include those available under the trade names Percumyl D (produced by NOF Corporation), Perhexa 3M (NOF Corporation), Perhexa C (NOF Corporation, and Luperco 231XL (Atochem Co.). The use of Perhexa 3M or Perhexa C is preferred.

A single organic peroxide may be used alone or two or more different organic peroxides may be mixed and used together. Mixing two or more different organic peroxides is preferred from the standpoint of further enhancing rebound.

The amount of the organic peroxide included per 100 parts of the base rubber is preferably at least 0.1 part by weight, more preferably at least 0.2 part by weight, and even more preferably at least 0.3 part by weight, but preferably not more than 2 parts by weight, more preferably not more than 1.5 parts by weight, and even more preferably not more than 1 part by weight. Including too much or too little organic peroxide may prevent the desired hardness profile from being achieved, making it impossible, in turn, to achieve the desired feel on impact, durability and rebound.

In the present invention, an antioxidant may be included if necessary. Illustrative examples of the antioxidant include commercial products such as Nocrac NS-6 and Nocrac NS-30 (both produced by Ouchi Shinko Chemical Industry Co., Ltd.), and Yoshinox 425 (Yoshitomi Pharmaceutical Industries, Ltd.).

To achieve a good rebound and durability, it is recommended that the amount of the antioxidant included per 100 parts by weight of the base rubber be preferably at least 0 part by weight, more preferably at least 0.03 part by weight, and even more preferably at least 0.05 part by weight, but prefer-

ably not more than 0.4 part by weight, more preferably not more than 0.3 part by weight, and even more preferably not more than 0.2 part by weight.

Sulfur may also be added if necessary. Such sulfur is exemplified by the product manufactured by Tsurumi Chemical Industry Co., Ltd. under the trade name "Sulfur Z." The amount of sulfur included per 100 parts by weight of the base rubber is preferably at least 0 part by weight, more preferably at least 0.005 part by weight, and more preferably at least 0.01 part by weight, but preferably not more than 0.5 part by weight, more preferably not more than 0.4 part by weight, and even more preferably not more than 0.1 part by weight. By adding sulfur, the core hardness profile can be increased. Adding too much sulfur may result in undesirable effects during hot molding, such as explosion of the rubber composition, or may considerably lower the rebound.

To achieve the subsequently described specific core center and surface hardnesses and deflections and the desired initial velocities (m/s), the foregoing rubber composition is suitably selected and fabrication of the solid core (hot-molded piece) is carried out by vulcanization and curing according to a method similar to that used for conventional golf ball rubber compositions. Suitable vulcanization conditions include, for example, a vulcanization temperature of between 100° C. and 200° C., and a vulcanization time of between 10 and 40 minutes. The vulcanization temperature is preferably at least 150° C., and especially at least 155° C., but preferably not above 200° C., more preferably not above 190° C., even more preferably not above 180° C., and most preferably not above 170° C.

The diameter of the solid core of the invention is not subject to any particular limitation. It is recommended that the solid core have a diameter of preferably at least 34.0 mm, more preferably at least 34.5 mm, even more preferably at least 35.0 mm, and most preferably at least 35.5 mm, but preferably not more than 38.7 mm, more preferably not more than 38.2 mm, even more preferably not more than 37.7 mm, and most preferably not more than 37.0 mm. At a small core diameter, the feel of the ball on impact may harden. On the other hand, at a large core diameter, the intermediate layer and cover necessarily become thinner, which may result in a poor durability.

The solid core has a center hardness, expressed as the Shore D hardness, of preferably at least 20, more preferably at least 25, even more preferably at least 30, and most preferably at least 35, but preferably not more than 45, more preferably not more than 44, even more preferably not more than 43, and most preferably not more than 42.

The surface of the solid core has a hardness, expressed as the Shore D hardness, of preferably at least 35, more preferably at least 39, even more preferably at least 41, and most preferably at least 43, but preferably not more than 65, more preferably not more than 60, even more preferably not more than 55, and most preferably not more than 53.

The hardness difference between the surface and center of the solid core as expressed in Shore D hardness units, while not subject to any particular limitation, is preferably at least 5, more preferably at least 6, and even more preferably at least 7, but preferably not more than 30, more preferably not more than 25, and even more preferably not more than 20. At a hardness difference smaller than the above range, the spin rate on shots with a driver may rise, lowering the distance traveled by the ball. On the other hand, at a hardness difference larger than the above range, the rebound and durability of the ball may decrease.

The solid core has a deflection, when compressed under a final load of 130 kgf from an initial load of 10 kgf, of prefer-

ably at least 3.0 mm, more preferably at least 3.3 mm, even more preferably at least 3.5 mm, and most preferably at least 3.7 mm, but preferably not more than 6.0 mm, more preferably not more than 5.5 mm, even more preferably not more than 5.0 mm, and most preferably not more than 4.8 mm. Too small a deflection by the solid core may worsen the feel of the ball on impact and, particularly on long shots such as with a driver in which the ball incurs a large deformation, may subject the ball to an excessive rise in the spin rate, shortening the distance traveled by the ball. On the other hand, a solid core which is too soft may deaden the feel of the ball when played and result in a less than adequate rebound, shortening the distance traveled by the ball, and moreover may give the ball a poor durability to cracking on repeated impact.

In the present invention, it is desirable to optimize the initial velocity of the core. The initial velocity of the core is preferably at least 76.0 m/s, more preferably at least 76.5 m/s, even more preferably at least 76.7 m/s, and most preferably at least 77.0 m/s, but preferably not more than 79.0 m/s, more preferably not more than 78.5 m/s, even more preferably not more than 78.0 m/s, and most preferably not more than 77.7 m/s. The core initial velocity is a value obtained by the same method of measurement as the method described in the subsequent examples. That is, it is a value measured using an initial velocity measuring apparatus of the same type as a USGA drum rotation-type initial velocity instrument approved by the R&A.

Next, in the present invention, various types of known thermoplastic resins may be used as the intermediate layer material. It is especially preferable to employ in the present invention an ionomer composition having one of the following base resins composed of components (a) to (c) below.

Base resin (I) composed of:

(a) from 95 to 50 wt % of an olefin-unsaturated carboxylic acid-unsaturated carboxylic acid ester random terpolymer and/or a metal salt thereof,

(b) from 0 to 10 wt % of an olefin-unsaturated carboxylic acid random copolymer and/or a metal salt thereof, and

(c) from 5 to 50 wt % of a thermoplastic block copolymer having a crystalline polyolefin block and a polyethylene/butylene random copolymer.

Base resin (II) composed of:

(a) from 0 to 20 wt % of an olefin-unsaturated carboxylic acid-unsaturated carboxylic acid ester random terpolymer and/or a metal salt thereof,

(b) from 95 to 50 wt % of an olefin-unsaturated carboxylic acid random copolymer and/or a metal salt thereof, and

(c) from 5 to 50 wt % of a thermoplastic block copolymer having a crystalline polyolefin block and a polyethylene/butylene random copolymer.

The olefin-unsaturated carboxylic acid-unsaturated carboxylic acid ester random terpolymer and/or a metal salt thereof serving as component (a) has a weight-average molecular weight (Mw) of preferably at least 100,000, more preferably at least 110,000, and even more preferably at least 120,000, but preferably not more than 200,000, more preferably not more than 190,000, and even more preferably not more than 170,000. The weight-average molecular weight (Mw) to number-average molecular weight (Mn) ratio for the copolymer is preferably from 3.0 to 7.0.

Above component (a) is an olefin-containing copolymer. The olefin in component (a) is exemplified by olefins in which the number of carbons is at least 2 but not more than 8, and preferably not more than 6. Illustrative examples of such olefins include ethylene, propylene, butene, pentene, hexene, heptene and octene. The use of ethylene is especially preferred.

Illustrative examples of the unsaturated carboxylic acid in component (a) include acrylic acid, methacrylic acid, maleic acid and fumaric acid. Acrylic acid and methacrylic acid are especially preferred.

5 The unsaturated carboxylic acid ester in component (a) may be, for example, a lower alkyl ester of an unsaturated carboxylic acid. Illustrative examples include methyl methacrylate, ethyl methacrylate, propyl methacrylate, butyl methacrylate, methyl acrylate, ethyl acrylate, propyl acrylate and butyl acrylate. The use of butyl acrylate (n-butyl acrylate, isobutyl acrylate) is especially preferred.

The random copolymer serving as component (a) in the invention may be obtained by the random copolymerization of the above ingredients in accordance with a known method.

15 It is recommended here that the unsaturated carboxylic acid content (acid content) within the random copolymer be generally at least 2 wt %, preferably at least 6 wt %, and more preferably at least 8 wt %, but not more than 25 wt %, preferably not more than 20 wt %, and more preferably not more than 15 wt %. At a low acid content, the rebound may decrease, whereas at a high acid content, the material processability may decrease.

20 The metal salt of the copolymer of component (a) may be obtained by neutralizing some of the acid groups in the random copolymer of component (a) with metal ions.

25 Examples of the metal ions which neutralize the acid groups include  $\text{Na}^+$ ,  $\text{K}^+$ ,  $\text{Li}^+$ ,  $\text{Zn}^{++}$ ,  $\text{Cu}^{++}$ ,  $\text{Mg}^{++}$ ,  $\text{Ca}^{++}$ ,  $\text{Co}^{++}$ ,  $\text{Ni}^{++}$  and  $\text{Pb}^{++}$ . Of these,  $\text{Na}^+$ ,  $\text{Li}^+$ ,  $\text{Zn}^{++}$ ,  $\text{Mg}^{++}$  or  $\text{Ca}^{++}$  are preferred, and  $\text{Zn}^{++}$  is especially preferred. The degree of

30 neutralization of the random copolymer by these metal ions, while not subject to any particular limitation, is generally at least 5 mol %, preferably at least 10 mol %, and especially at least 20 mol %, but not more than 95 mol %, preferably not more than 90 mol %, and especially not more than 80 mol %.

35 At a degree of neutralization in excess of 95 mol %, the moldability may decrease. On the other hand, at less than 5 mol %, there arises a need to increase the amount in which the inorganic metal compound serving as component (c) is added, which may present a drawback in terms of cost. Such a neutralization product may be obtained by a known method. For example, the neutralization product may be obtained by introducing a metal ion compound, such as a formate, acetate, nitrate, carbonate, bicarbonate, oxide, hydroxide or alkoxide, into the random copolymer.

40 45 Illustrative examples of the olefin-unsaturated carboxylic acid-unsaturated carboxylic acid ester random terpolymer serving as component (a) include those available under the trade names Nucrel AN4318, Nucrel AN4319, and Nucrel AN4311 (DuPont-Mitsui Polymers Co., Ltd.). Illustrative examples of the metal salts of olefin-unsaturated car-

50 boxylic acid-unsaturated carboxylic acid ester random terpolymer include those available under the trade names Himilan AM7316, Himilan AM7331, Himilan 1855 and Himilan 1856 (DuPont-Mitsui Polymers Co., Ltd.), and

55 those available under the trade names Surlyn 6320 and Surlyn 8120 (E.I. DuPont de Nemours and Co., Ltd.).

The olefin-unsaturated carboxylic acid random copolymer and/or metal salt serving as component (b) has a weight-average molecular weight (Mw) of preferably between 100,000 and 200,000, more preferably between 110,000 and 190,000, and even more preferably between 120,000 and 170,000. The weight-average molecular weight (Mw) to number-average molecular weight (Mn) ratio for the copolymer is preferably from 3.0 to 7.0.

60 65 Illustrative examples of the olefin-unsaturated carboxylic acid random copolymer serving as component (b) include those available under the trade names Nucrel 1560, Nucrel

1525 and Nucrel 1035 (DuPont-Mitsui Polymers Co., Ltd.). Illustrative examples of the metal salts of olefin-unsaturated carboxylic acid binary random copolymer include those available under the trade names Himilan 1605, Himilan 1601, Himilan 1557, Himilan 1705 and Himilan 1706 (DuPont-Mitsui Polymers Co., Ltd.) and those available under the trade names Surlyn 7930 and Surlyn 7920 (E.I. DuPont de Nemours and Co., Ltd.).

The thermoplastic block copolymer having a crystalline polyolefin block and a polyethylene/butylene random copolymer which serves as component (c) is exemplified by thermoplastic block copolymers composed of crystalline polyethylene blocks (E) as hard segments and blocks of a relatively random copolymer of ethylene and butylene (EB) as soft segments. Preferred use may be made of block copolymers having a molecular structure with a hard segment at one or both ends, such as block copolymers having an E-EB or E-EB-E structure.

Such thermoplastic block copolymers having a crystalline polyolefin block and a polyethylene/butylene random copolymer which serve as component (c) may be obtained by hydrogenating polybutadiene.

A polybutadiene in which bonding within the butadiene structure is characterized by the presence of a block-like 1,4-polymer region having a 1,4-bond content of from 95 to 100 wt %, and in which the butadiene structure as a whole has a 1,4-bond content of from 50 to 100 wt %, and preferably from 80 to 100 wt %, may be suitably used here as the polybutadiene subjected to hydrogenation. That is, preferred use may be made of a polybutadiene having a 1,4-bond content of 50 to 100 wt %, and preferably 80 to 100 wt %, and having a block-like 1,4-polymer region with a 1,4-bond content of 95 to 100 wt %.

The above-mentioned E-EB-E type thermoplastic block copolymer is preferably one obtained by hydrogenating a polybutadiene having at both ends of the molecular chain 1,4-polymerization products which are rich in 1,4-bonds and having an intermediate region where 1,4-bonds and 1,2-bonds are intermingled. The degree of hydrogenation (conversion of double bonds on the polybutadiene to saturated bonds) in the polybutadiene hydrogenate is preferably from 60 to 100%, and more preferably from 90 to 100%. Too low a degree of hydrogenation may give rise to undesirable effects such as gelation in the blending step with other components such as an ionomer resin and, when the golf ball is formed, may lead to problems associated with the intermediate layer, such as a poor durability to impact.

In the block copolymer having a E-EB or E-EB-E molecular structure with a hard segment at one or both ends that may be preferably used as the thermoplastic block copolymer, the content of the hard segments is preferably from 10 to 50 wt %. If the content of hard segments is too high, the intermediate layer may lack sufficient softness, making it difficult to effectively achieve the objects of the invention. On the other hand, if the content of hard segments is too low, the blend may have a poor moldability.

The thermoplastic block copolymer has a melt index, at 230° C. and a test load of 21.2 N, of preferably from 0.01 to 15 g/10 min, and more preferably from 0.03 to 10 g/10 min. Outside of this range, problems such as weld lines, sink marks and short shots may arise during injection molding.

Moreover, the thermoplastic block copolymer preferably has a surface hardness of from 10 to 50. If the surface hardness is too low, the golf ball may have a decreased durability to repeated impact. On the other hand, if the surface hardness is too high, blends of the thermoplastic block with an ionomer resin may have a decreased rebound.

The thermoplastic block copolymer has a number-average molecular weight of preferably between 30,000 and 800,000.

Commercial products may be used as the above-described thermoplastic block copolymer having a crystalline polyolefin block and a polyethylene/butylene random copolymer. Illustrative examples include Dynaron 6100P, Dynaron 6200P and Dynaron 6201B available from JSR Corporation. Dynaron 6100P, which is a block polymer having crystalline olefin blocks at both ends, is especially preferred for use in the present invention. These olefin thermoplastic elastomers may be used singly or as mixtures of two or more thereof.

The proportion of the overall base resin accounted for by the copolymer serving as component (c) is preferably at least 5 wt %, more preferably at least 8 wt %, even more preferably at least 11 wt %, and most preferably at least 14 wt %, but preferably not more than 50 wt %, more preferably not more than 40 wt %, even more preferably not more than 30 wt %, and most preferably not more than 20 wt %.

The intermediate layer material also includes, mixed 20 therein per 100 parts by weight of above resin components (a) to (c):

(d) from 5 to 100 parts by weight of a fatty acid or fatty acid derivative having a molecular weight of from 280 to 1500; and

(e) from 0.1 to 10 parts by weight of a basic inorganic metal compound capable of neutralizing acid groups within components (a), (b) and (d).

Component (d) is a fatty acid or fatty acid derivative having a molecular weight of at least 280 but not more than 1500 30 whose purpose is to enhance the flow properties of the heated mixture. It has a molecular weight which is much smaller than those of components (a) to (c), and helps to significantly decrease the melt viscosity of the mixture. Also, because the fatty acid (or fatty acid derivative) of component (d) has a molecular weight of at least 280 but not more than 1500 and has a high content of acid groups (or derivative moieties thereof), its addition to the resin material results in little if any loss of rebound.

The fatty acid or fatty acid derivative serving as component 40 (d) may be an unsaturated fatty acid or fatty acid derivative having a double bond or triple bond in the alkyl moiety, or it may be a saturated fatty acid or fatty acid derivative in which all the bonds in the alkyl moiety are single bonds. It is recommended that the number of carbon atoms on the molecule 45 be preferably at least 18, but preferably not more than 80, and more preferably not more than 40. Too few carbons may result in a poor heat resistance, and may also set the acid group content so high as to cause the acid groups to interact with acid groups present on the base resin, diminishing the flow-improving effects. On the other hand, too many carbons increases the molecular weight, which may significantly lower the flow properties, and make the material difficult to use.

Specific examples of fatty acids that may be used as component (d) include stearic acid, 12-hydroxystearic acid, behenic acid, oleic acid, linoleic acid, linolenic acid, arachidic acid and lignoceric acid. Of these, preferred use 55 may be made of stearic acid, arachidic acid, behenic acid and lignoceric acid.

The fatty acid derivative of component (d) is exemplified by derivatives in which the proton on the acid group of the fatty acid has been substituted. Exemplary fatty acid derivatives of this type include metallic soaps in which the proton has been substituted with a metal ion. Metal ions that may be used in such metallic soaps include  $\text{Li}^+$ ,  $\text{Ca}^{++}$ ,  $\text{Mg}^{++}$ ,  $\text{Zn}^{++}$ ,  $\text{Mn}^{++}$ ,  $\text{Al}^{+++}$ ,  $\text{Ni}^{++}$ ,  $\text{Fe}^{++}$ ,  $\text{Fe}^{+++}$ ,  $\text{Cu}^{++}$ ,  $\text{Sn}^{++}$ ,  $\text{Pb}^{++}$  and  $\text{Co}^{++}$ . Of these,  $\text{Ca}^{++}$ ,  $\text{Mg}^{++}$  and  $\text{Zn}^{++}$  are especially preferred.

## 11

Specific examples of fatty acid derivatives that may be used as component (d) include magnesium stearate, calcium stearate, zinc stearate, magnesium 12-hydroxystearate, calcium 12-hydroxystearate, zinc 12-hydroxystearate, magnesium arachidate, calcium arachidate, zinc arachidate, magnesium behenate, calcium behenate, zinc behenate, magnesium lignocerate, calcium lignocerate and zinc lignocerate. Of these, magnesium stearate, calcium stearate, zinc stearate, magnesium arachidate, calcium arachidate, zinc arachidate, magnesium behenate, calcium behenate, zinc behenate, magnesium lignocerate, calcium lignocerate and zinc lignocerate are preferred.

In the present invention, the amount of component (d) used per 100 parts by weight of the base resin is at least 5 parts by weight, preferably at least 8 parts by weight, more preferably at least 20 parts by weight, and even more preferably at least 40 parts by weight, but not more than 100 parts by weight, preferably not more than 90 parts by weight, even more preferably not more than 80 parts by weight, and most preferably not more than 70 parts by weight.

Use may also be made of known metallic soap-modified ionomers (see, for example, U.S. Pat. No. 5,312,857, U.S. Pat. No. 5,306,760 and International Disclosure WO 98/46671) when using above components (a) and (b).

Component (e) is a basic inorganic metal compound capable of neutralizing the acid groups in above components (a), (b) and (d). As mentioned in prior-art examples, when components (a), (b) and (d) alone, and in particular a metal-modified ionomer resin alone (e.g., a metal soap-modified ionomer resin of the type mentioned in the foregoing patent publications, alone), are heated and mixed, as shown below, the metallic soap and un-neutralized acid groups present on the ionomer undergo exchange reactions, generating a fatty acid. Because the fatty acid has a low thermal stability and readily vaporizes during molding, it causes molding defects. Moreover, if the fatty acid thus generated deposits on the surface of the molded material, it substantially lowers paint film adhesion. Component (e) is included so as to resolve such problems.



The heated mixture used in the present invention thus includes, as component (e), a basic inorganic metal compound which neutralizes the acid groups present in above components (a), (b) and (d). The inclusion of component (e) as an essential ingredient confers excellent properties. That is, the acid groups in above components (a), (b) and (d) are neutralized, and synergistic effects from the inclusion of each of these components increase the thermal stability of the heated mixture while at the same time conferring a good moldability and enhancing the rebound of the golf ball.

It is recommended that above component (e) be a basic inorganic metal compound—preferably a monoxide or hydroxide—which is capable of neutralizing acid groups in above components (a), (b) and (d). Because such compounds

## 12

have a high reactivity with the ionomer resin and the reaction by-products contain no organic matter, the degree of neutralization of the heated mixture can be increased without a loss of thermal stability.

The metal ions used here in the basic inorganic metal compound are exemplified by  $\text{Li}^+$ ,  $\text{Na}^+$ ,  $\text{K}^+$ ,  $\text{Ca}^{++}$ ,  $\text{Mg}^{++}$ ,  $\text{Zn}^{++}$ ,  $\text{Al}^{+++}$ ,  $\text{Ni}^+$ ,  $\text{Fe}^{++}$ ,  $\text{Fe}^{+++}$ ,  $\text{Cu}^{++}$ ,  $\text{Mn}^{++}$ ,  $\text{Sn}^{++}$ ,  $\text{Pb}^{++}$  and  $\text{Co}^{++}$ . Illustrative examples of the inorganic metal compound include basic inorganic fillers containing these metal ions, such as magnesium oxide, magnesium hydroxide, magnesium carbonate, zinc oxide, sodium hydroxide, sodium carbonate, calcium oxide, calcium hydroxide, lithium hydroxide and lithium carbonate. As noted above, a monoxide or hydroxide is preferred. The use of magnesium oxide or calcium hydroxide, which have high reactivities with ionomer resins, is especially preferred.

Component (e) of the present invention is included in an amount, per 100 parts by weight of the base resin, of from 0.1 to 10 parts by weight, preferably at least 0.5 part by weight, more preferably at least 1 part by weight, but preferably not more than 5 parts by weight, more preferably not more than 3 parts by weight.

The heated mixture used in the present invention, which includes, as described above, components (a) to (e), can be provided with improved thermal stability, moldability and resilience. To this end, it is recommended that, in all heated mixtures used in the invention, at least 70 mol %, preferably at least 80 mol %, and more preferably at least 90 mol %, of the acid groups in the mixture be neutralized. A high degree of neutralization more reliably suppresses the exchange reactions that pose a problem in the above-described cases where components (a) and (b) and the fatty acid (or fatty acid derivative) alone are used, thus making it possible to prevent the generation of fatty acids. As a result, a material can be obtained which has a markedly increased thermal stability, a good moldability, and a substantially higher resilience than conventional ionomer resins.

Here, with regard to neutralization of the heated mixture of the invention, to more reliably achieve both a high degree of neutralization and good flow properties, it is recommended that the acid groups in the heated mixture be neutralized with transition metal ions and with alkali metal and/or alkaline earth metal ions. Because transition metal ions have a weaker ionic cohesion than alkali metal and alkaline earth metal ions, it is possible in this way to neutralize some of the acid groups in the heated mixture and thus enable the flow properties to be significantly improved.

In the present invention, various additives may also be optionally included in the above heated mixture. Additives which may be used include pigments, dispersants, antioxidants, ultraviolet absorbers and optical stabilizers. Moreover, to improve the feel of the golf ball on impact, the resin composition may also include, in addition to the above essential ingredients, various non-ionomeric thermoplastic elastomers. Illustrative examples of such non-ionomeric thermoplastic elastomers include styrene-based thermoplastic elastomers, ester-based thermoplastic elastomers and urethane-based thermoplastic elastomers. The use of styrene-based thermoplastic elastomers is especially preferred.

The method of preparing the heated mixture is exemplified by mixture under heating at a temperature of between 150 and 250°C. in an internal mixer such as a twin-screw extruder, a Banbury mixer or a kneader. The method of forming the intermediate layer using the heated mixture is not subject to any particular limitation. For example, the intermediate layer may be formed by injection molding or compression molding the heated mixture. When injection molding is employed, the

process may involve placing a prefabricated solid core at a given position in the injection mold, then introducing the above-described material into the mold. When compression molding is employed, the process may involve producing a pair of half cups from the above-described material, covering the core with these half-cups, either directly or with an intervening intermediate layer, then applying pressure and heat within a mold. If molding under heat and pressure is carried out, the molding conditions may be a temperature of from 120 to 170° C. and a period of from 1 to 5 minutes.

The intermediate layer material in the invention has a hardness which, while not subject to any particular limitation, is preferably at least 35, more preferably at least 40, even more preferably at least 43, and most preferably at least 46, but preferably not more than 57, more preferably not more than 55, even more preferably not more than 53, and most preferably not more than 52. If the Shore D hardness is low, the rebound may decrease, resulting in a shorter distance.

It is recommended that the intermediate layer be formed to a thickness which, while not subject to any particular limitation, is preferably at least 1.0 mm, more preferably at least 1.2 mm, even more preferably at least 1.4, and even more preferably at least 1.6 mm, but preferably not more than 2.5 mm, preferably not more than 2.3 mm, even more preferably not more than 2.2 mm, and most preferably not more than 2.1 mm. If the intermediate layer is too thick, it will not be possible to enhance the feel and the distance and flight performance of the ball. On the other hand, if the intermediate layer is too thin, the distance and flight performance and the durability will worsen.

The intermediate layer material has a melt flow rate (measured in accordance with JIS-K6760 (test temperature, 190° C.; test load, 21 N (2.16 kgf)) of preferably at least 9 g/10 min, more preferably at least 10 g/10 min, even more preferably at least 11 g/10 min, and most preferably at least 12 g/10 min, but preferably not more than 30 g/10 min, more preferably not more than 25 g/10 min, even more preferably not more than 21 g/10 min, and most preferably not more than 18 g/10 min. If the melt index of the heated mixture is low, the processability of the mixture may markedly decrease.

Also, in the present invention, it is desirable that the Shore D hardness of the intermediate layer minus the Shore D hardness of the solid core surface be within  $\pm 10$ . The upper limit of this hardness difference is preferably 8 or less, more preferably 6 or less, and most preferably 5 or less, and the lower limit is preferably at least -7, more preferably at least -4, and even more preferably at least -1. When this hardness difference is above 10, the intermediate layer is too hard and the core is too soft, detracting from the feel of the ball and lowering the rebound and durability. On the other hand, when the hardness difference is below -10, the intermediate layer is too soft and the core is too hard, detracting from the feel of the ball on impact and lowering the ball rebound.

In the present invention, the sphere I composed of the core encased by the intermediate layer has a deflection (mm), when compressed under a final load of 130 kgf from an initial load of 10 kgf, of preferably at least 2.0 mm, more preferably at least 2.2 mm, even more preferably at least 2.4 mm, and most preferably at least 2.6 mm, but preferably not more than 5.5 mm, more preferably not more than 5.0 mm, even more preferably not more than 4.5 mm, and most preferably not more than 4.0 mm. Outside of this range, the ball may have a poor feel on impact, or may have a poor distance.

In the present invention, the sphere I composed of the core encased by the intermediate layer has an initial velocity of preferably at least 76.0 m/s, more preferably at least 76.5 m/s, even more preferably at least 76.7 m/s, and most preferably at

least 77.0 m/s, but preferably not more than 78.5 m/s, more preferably not more than 78.3 m/s, even more preferably not more than 78.0 m/s, and most preferably not more than 77.7 m/s. The initial velocity of the sphere I, which is defined in the same way as the definition of the initial velocity of the core, is a value obtained by the same method of measurement as the methods described in the subsequent examples. That is, it is a value measured using an initial velocity measuring apparatus of the same type as a USGA drum rotation-type initial velocity instrument approved by the R&A.

Next, the cover used in the present invention is described. In the present invention, a thermoplastic resin material is used as the cover material. The thermoplastic resin is not subject to any particular limitation. However, from the standpoint of comprehensively achieving the effects of the invention, the cover material is preferably a thermoplastic ionomer or a polyurethane. Thermoplastic ionomers that may be employed include commercially available ionomers, and also the ionomeric compositions described above in connection with the intermediate layer material. When a polyurethane is employed as the cover material, the following applies.

#### When a Polyurethane is Used

When the cover material is made primarily of a thermoplastic polyurethane, golf balls having an excellent scuff resistance and an excellent spin stability on shots known as "fliers" can be obtained.

The thermoplastic polyurethane is not subject to any particular limitation, provided it is a thermoplastic elastomer composed primarily of polyurethane. However, thermoplastic polyurethanes with a structure that includes soft segments made of a high-molecular-weight polyol compound and hard segments made of a chain extender and a diisocyanate are preferred.

Any high-molecular-weight polyol compound employed in the prior art relating to thermoplastic polyurethane materials may be used without particular limitation. Preferred examples include polyester polyols, polyether polyols, copolyester polyols and polycarbonate polyols. Of these, polyether polyols are preferred for the preparation of thermoplastic polyurethanes having excellent rebound resilience and low-temperature properties, and polyester polyols are preferred for the heat resistance and broad molecular design capabilities they provide.

Any diisocyanate employed in the prior art relating to thermoplastic polyurethane materials may be used without particular limitation. Illustrative examples include 4,4'-diphenylmethane diisocyanate, 2,4-toluene diisocyanate, 2,6-toluene diisocyanate, xylylene diisocyanate, 1,5-naphthylene diisocyanate, tetramethylxylene diisocyanate, hydrogenated xylylene diisocyanate, dicyclohexylmethane diisocyanate, tetramethylene diisocyanate, hexamethylene diisocyanate, isophorone diisocyanate, norbornene diisocyanate, dimer acid diisocyanate, 2,2,4- and 2,4,4-trimethylhexamethylene diisocyanate and lysine diisocyanate. However, depending on the type of isocyanate, the crosslinking reaction during injection molding may be difficult to control. In the practice of the invention, the use of 4,4'-diphenylmethane diisocyanate is preferred for good compatibility with the subsequently described isocyanate mixture.

Any chain extender employed in the prior art relating to thermoplastic polyurethane materials may be used without particular limitation. For instance, use may be made of any ordinary polyol or polyamine. Specific examples include 1,4-butyleneglycol, 1,2-ethylene glycol, 1,3-butanediol, 1,6-hexanediol, 2,2-dimethyl-1,3-propanediol, dicyclohexylmethylenediamine (hydrogenated MDI) and isophoronediamine (IPDA). These chain extenders have a

## 15

number-average molecular weight of generally at least 20, but generally not more than 15,000.

No limitation is imposed on the specific gravity of the thermoplastic polyurethane, so long as it is suitably adjusted within a range that allows the objects of the invention to be achieved. The specific gravity is preferably at least 1.0, and more preferably at least 1.1, but preferably not more than 1.3, and more preferably not more than 1.25.

The thermoplastic polyurethane used in the invention may be a commercial product. Illustrative examples include Pandex T8290, Pandex T8295 and Pandex T8260 (all manufactured by DIC Bayer Polymer, Ltd.), and Resamine 2593 and Resamine 2597 (both manufactured by Dainichi Seika Colour & Chemicals Mfg. Co., Ltd.).

The resin which forms the cover may be composed of the above-described thermoplastic polyurethane. A type of polyurethane in which the molecule has a partially crosslinked structure is preferred. The use of at least one type selected from the following two types of polyurethanes (first polyurethane, second polyurethane) is especially preferred for further enhancing the scuff resistance.

## First Polyurethane

A thermoplastic polyurethane composition composed of the above-described thermoplastic polyurethane (A) and an isocyanate mixture (B) is used.

The isocyanate mixture (B) is preferably one prepared by dispersing (b-1) a compound having as functional groups at least two isocyanate groups per molecule in (b-2) a thermoplastic resin that is substantially non-reactive with isocyanate. The compound having as functional groups at least two isocyanate groups per molecule which serves as component (b-1) may be an isocyanate compound used in the prior art relating to polyurethanes, examples of which include aromatic isocyanates, hydrogenated aromatic isocyanates, aliphatic diisocyanates and alicyclic diisocyanates. Specific examples include isocyanate compounds such as those mentioned above. From the standpoint of reactivity and work safety, the use of 4,4'-diphenylmethane diisocyanate is preferred.

The thermoplastic resin that is substantially non-reactive with isocyanate which serves as component (b-2) is preferably a resin having a low water absorption and excellent compatibility with thermoplastic polyurethane materials. Illustrative, non-limiting, examples of such resins include polystyrene resins, polyvinyl chloride resins, ABS resins, polycarbonate resins and polyester thermoplastic elastomers (e.g., polyether-ester block copolymers, polyester-ester block copolymers).

For good rebound resilience and strength, the use of a polyester thermoplastic elastomer is especially preferred. No particular limitation is imposed on the polyester thermoplastic elastomer, provided it is a thermoplastic elastomer composed primarily of polyester. The use of a polyester-based block copolymer composed primarily of high-melting crystalline polymer segments made of crystalline aromatic polyester units and low-melting polymer segments made of aliphatic polyether units and/or aliphatic polyester units is preferred. In addition, up to 5 mol % of polycarboxylic acid ingredients, polyoxy ingredients and polyhydroxy ingredients having a functionality of three or more may be copolymerized. In the low-melting polymer segments made of aliphatic polyether units and/or aliphatic polyester units, illustrative examples of the aliphatic polyether include poly(ethylene oxide) glycol, poly(propylene oxide) glycol, poly(tetramethylene oxide) glycol, poly(hexamethylene oxide) glycol, copolymers of ethylene oxide and propylene oxide, ethylene oxide addition polymers of poly(propylene oxide)

## 16

glycols, and copolymers of ethylene oxide and tetrahydrofuran. Illustrative examples of the aliphatic polyester include poly( $\epsilon$ -caprolactone), polyanantholactone, polycaprylolactone, poly(butylene adipate) and poly(ethylene adipate).

5 Examples of polyester thermoplastic elastomers preferred for use in the invention include those in the Hytrel series made by DuPont-Toray Co., Ltd., and those in the Primalloy series made by Mitsubishi Chemical Corporation.

When the isocyanate mixture (B) is prepared, it is desirable 10 for the relative proportions of above components (b-1) and (b-2), expressed as the weight ratio (b-1)/(b-2), to be within a range of 100/5 to 100/100, and especially 100/10 to 100/40. If the amount of component (b-1) relative to component (b-2) is 15 too low, more isocyanate mixture (B) must be added to achieve an amount of addition adequate for the crosslinking reaction with the thermoplastic polyurethane (A). In such cases, component (b-2) exerts a large influence, which may diminish the physical properties of the thermoplastic polyurethane composition serving as the cover material. If, on the other hand, the amount of component (b-1) is too high, component (b-1) may cause slippage to occur during mixing, 20 making it difficult to prepare the thermoplastic polyurethane composition used as the cover material.

The isocyanate mixture (B) can be prepared by blending 25 component (b-1) into component (b-2) and thoroughly working together these components at a temperature of 130 to 250° C. using a mixing roll mill or a Banbury mixer, then either pelletizing or cooling and grinding. The isocyanate mixture (B) used may be a commercial product, a preferred example 30 of which is Crossnate EM30 (made by Dainichi Seika Colour & Chemicals Mfg. Co., Ltd.). Above component (B) is included in an amount, per 100 parts by weight of component (A), of generally at least 1 part by weight, preferably at least 5 parts by weight, and more preferably at least 10 parts by 35 weight, but generally not more than 100 parts by weight, preferably not more than 50 parts by weight, and more preferably not more than 30 parts by weight. Too little component (B) may make it impossible to achieve a sufficient crosslinking reaction, so that there is no apparent enhancement of the 40 physical properties. On the other hand, too much may result in greater discoloration over time or due to the effects of heat and ultraviolet light, and may also have other undesirable effects, such as lowering the rebound.

## Second Polyurethane

45 At least one cover layer is made of a molded resin composition consisting primarily of (A) a thermoplastic polyurethane and (B) a polyisocyanate compound. The resin composition has present therein a polyisocyanate compound within at least a portion of which all the isocyanate groups on the molecule remain in an unreacted state. Golf balls made with such a thermoplastic polyurethane have an excellent rebound, spin performance and scuff resistance.

The cover layer is composed mainly of a thermoplastic polyurethane, and is formed of a resin composition of primarily (A) a thermoplastic polyurethane and (B) a polyisocyanate compound.

To fully exhibit the advantageous effects of the invention, a necessary and sufficient amount of unreacted isocyanate groups should be present in the cover-forming resin material. 60 Specifically, it is recommended that the combined weight of above components A and B together be at least 60%, and preferably at least 70%, of the total weight of the cover layer. Components A and B are described in detail below.

The thermoplastic polyurethane serving as component A 65 has a structure which includes soft segments made of a polymeric polyol(polymeric glycol) that is a long-chain polyol, and hard segments made of a chain extender and a polyiso-

cyanate compound. Here, the long-chain polyol used as a starting material is not subject to any particular limitation, and may be any that is used in the prior art relating to thermoplastic polyurethanes. Exemplary long-chain polyols include polyester polyols, polyether polyols, polycarbonate polyols, polyester polycarbonate polyols, polyolefin polyols, conjugated diene polymer-based polyols, castor oil-based polyols, silicone-based polyols and vinyl polymer-based polyols. These long-chain polyols may be used singly or as combinations of two or more thereof. Of the long-chain polyols mentioned here, polyether polyols are preferred because they enable the synthesis of thermoplastic polyurethanes having a high rebound resilience and excellent low-temperature properties.

Illustrative examples of the above polyether polyol include poly(ethylene glycol), poly(propylene glycol), poly(tetramethylene glycol) and poly(methyltetramethylene glycol) obtained by the ring-opening polymerization of a cyclic ether. The polyether polyol may be used singly or as a combination of two or more thereof. Of these, poly(tetramethylene glycol) and/or poly(methyltetramethylene glycol) are preferred.

It is preferable for these long-chain polyols to have a number-average molecular weight in a range of 1,500 to 5,000. By using a long-chain polyol having a number-average molecular weight within this range, a golf ball which is composed of a thermoplastic polyurethane composition and has excellent properties such as rebound and manufacturability can be reliably obtained. The number-average molecular weight of the long-chain polyol is more preferably in a range of 1,700 to 4,000, and even more preferably in a range of 1,900 to 3,000.

As used herein, "number-average molecular weight of the long-chain polyol" refers to the number-average molecular weight computed based on the hydroxyl number measured in accordance with JIS K-1557.

Suitable chain extenders include those used in the prior art relating to thermoplastic polyurethanes. For example, low-molecular-weight compounds which have a molecular weight of 400 or less and include on the molecule two or more active hydrogen atoms capable of reacting with isocyanate groups are preferred. Illustrative, non-limiting, examples of the chain extender include 1,4-butylene glycol, 1,2-ethylene glycol, 1,3-butanediol, 1,6-hexanediol and 2,2-dimethyl-1,3-propanediol. Of these chain extenders, aliphatic diols having 2 to 12 carbons are preferred, and 1,4-butylene glycol is especially preferred.

The polyisocyanate compound is not subject to any particular limitation, although use may be made of one that is used in the prior art relating to thermoplastic polyurethanes. Specific examples include one or more selected from the group consisting of 4,4'-diphenylmethane diisocyanate, 2,4-toluene diisocyanate, 2,6-toluene diisocyanate, p-phenylene diisocyanate, xylylene diisocyanate, naphthylene-1,5-diisocyanate, tetramethylxylene diisocyanate, hydrogenated xylylene diisocyanate, dicyclohexylmethane diisocyanate, tetramethylene diisocyanate, hexamethylene diisocyanate, isophorone diisocyanate, norbornene diisocyanate, trimethylhexamethylene diisocyanate and dimer acid diisocyanate. Depending on the type of isocyanate used, the crosslinking reaction during injection molding may be difficult to control. In the practice of the invention, to provide a balance between stability at the time of production and the properties that are manifested, it is most preferable to use 4,4'-diphenylmethane diisocyanate, which is an aromatic diisocyanate.

It is most preferable for the thermoplastic polyurethane serving as above component A to be a thermoplastic polyurethane synthesized using a polyether polyol as the long-chain polyol, using an aliphatic diol as the chain extender, and using

an aromatic diisocyanate as the polyisocyanate compound. It is desirable, though not essential, for the polyether polyol to be a polytetramethylene glycol having a number-average molecular weight of at least 1,900, for the chain extender to be 1,4-butylene glycol, and for the aromatic diisocyanate to be 4,4'-diphenylmethane diisocyanate.

The mixing ratio of activated hydrogen atoms to isocyanate groups in the above polyurethane-forming reaction can be adjusted within a desirable range so as to make it possible to obtain a golf ball which is composed of a thermoplastic polyurethane composition and has various improved properties, such as rebound, spin performance, scuff resistance and manufacturability. Specifically, in preparing a thermoplastic polyurethane by reacting the above long-chain polyol, polyisocyanate compound and chain extender, it is desirable to use the respective components in proportions such that the amount of isocyanate groups on the polyisocyanate compound per mole of active hydrogen atoms on the long-chain polyol and the chain extender is from 0.95 to 1.05 moles.

No particular limitation is imposed on the method of preparing the thermoplastic polyurethane used as component A. Production may be carried out by either a prepolymer process or one-shot process in which the long-chain polyol, chain extender and polyisocyanate compound are used and a known urethane-forming reaction is effected. Of these, a process in which melt polymerization is carried out in a substantially solvent-free state is preferred. Production by continuous melt polymerization using a multiple screw extruder is especially preferred.

Illustrative examples of the thermoplastic polyurethane serving as component A include commercial products such as Pandex T8295, Pandex T8290 and Pandex T8260 (all available from DIC Bayer Polymer, Ltd.).

Next, concerning the polyisocyanate compound used as component B, it is necessary that, in at least some of the polyisocyanate compound in the single resin composition, all the isocyanate groups on the molecule remain in an unreacted state. That is, polyisocyanate compound in which all the isocyanate groups on the molecule are in a completely free state must be present within the single resin composition, and such a polyisocyanate compound may be present together with polyisocyanate compound in which some of the isocyanate groups on the molecule are in a free state.

Various types of isocyanates may be employed without particular limitation as this polyisocyanate compound. Illustrative examples include one or more selected from the group consisting of 4,4'-diphenylmethane diisocyanate, 2,4-toluene diisocyanate, 2,6-toluene diisocyanate, p-phenylene diisocyanate, xylylene diisocyanate, naphthylene-1,5-diisocyanate, tetramethylxylene diisocyanate, hydrogenated xylylene diisocyanate, dicyclohexylmethane diisocyanate, tetramethylene diisocyanate, hexamethylene diisocyanate, isophorone diisocyanate, norbornene diisocyanate, trimethylhexamethylene diisocyanate and dimer acid diisocyanate. Of the above group of isocyanates, the use of 4,4'-diphenylmethane diisocyanate, dicyclohexylmethane diisocyanate and isophorone diisocyanate is preferable for achieving a good balance between the influence on moldability of such effects as the rise in viscosity that accompanies the reaction with the thermoplastic polyurethane serving as component A and the physical properties of the resulting golf ball cover material.

In the practice of the invention, although not an essential constituent, a thermoplastic elastomer other than the above-described thermoplastic polyurethane may be included as component C together with components A and B. Including this component C in the above resin composition enables the flow properties of the resin composition to be further

19

improved and enables various properties required of golf ball cover materials, such as resilience and scuff resistance, to be increased.

Component C, which is a thermoplastic elastomer other than the above thermoplastic polyurethane, is exemplified by one or more thermoplastic elastomer selected from among polyester elastomers, polyamide elastomers, ionomer resins, styrene block elastomers, hydrogenated styrene-butadiene rubbers, styrene-ethylene/butylene-ethylene block copolymers and modified forms thereof, ethylene-ethylene/butylene-ethylene block copolymers and modified forms thereof, styrene-ethylene/butylene-styrene block copolymers and modified forms thereof, ABS resins, polyacetals, polyethylenes and nylon resins. The use of polyester elastomers, polyamide elastomers and polyacetals is especially preferred because, owing to reactions with isocyanate groups, the resilience and scuff resistance are enhanced while retaining a good manufacturability.

The relative proportions of above components A, B and C are not subject to any particular limitation, although to fully achieve the advantageous effects of the invention, it is preferable for the weight ratio A:B:C of the respective components to be from 100:2:50 to 100:50:0, and more preferably from 100:2:50 to 100:30:8.

In the practice of the invention, the resin composition is prepared by mixing component A with component B, and additionally mixing in also component C. It is critical to select the mixing conditions such that, of the polyisocyanate compound, at least some polyisocyanate compound is present in which all the isocyanate groups on the molecule remain in an unreacted state. For example, treatment such as mixture in an inert gas (e.g., nitrogen) or in a vacuum state must be furnished. The resin composition is then injection-molded around a core which has been placed in a mold. To smoothly and easily handle the resin composition, it is preferable for the composition to be formed into pellets having a length of 1 to 10 mm and a diameter of 0.5 to 5 mm. Isocyanate groups in an unreacted state remain in these resin pellets; the unreacted isocyanate groups react with component A or component C to form a crosslinked material while the resin composition is being injection-molded about the core, or due to post-treatment such as annealing.

The above method of molding the cover is exemplified by feeding the above-described resin composition to an injection molding machine, and injecting the molten resin composition around the core so as to form a cover layer. The molding temperature varies according to such factors as the type of thermoplastic polyurethane, but is preferably in a range of 150 to 250° C.

When injection molding is carried out, it is desirable though not essential to carry out molding in a low-humidity environment such as by purging with a low-temperature gas using an inert gas such as nitrogen or low dew-point dry air or by vacuum treating some or all places on the resin paths from the resin feed area to the mold interior. Illustrative, non-limiting examples of the medium used for transporting the resin include low-moisture gases such as low dew-point dry air or nitrogen. By carrying out molding in such a low-humidity environment, reaction by the isocyanate groups is kept from proceeding before the resin has been charged into the mold interior. As a result, polyisocyanate in which the isocyanate groups are present in an unreacted state is included to some degree in the resin molded part, thus making it possible to reduce variable factors such as an unwanted rise in viscosity and enabling the effective crosslinking efficiency to be enhanced.

20

Techniques that can be used to confirm the presence of polyisocyanate compound in an unreacted state within the resin composition prior to injection molding about the core include those which involve extraction with a suitable solvent that selectively dissolves out only the polyisocyanate compound. An example of a simple and convenient method is one in which confirmation is carried out by simultaneous thermogravimetric and differential thermal analysis (TG-DTA) measurement in an inert atmosphere. For example, when the resin composition (cover material) used in the invention is heated in a nitrogen atmosphere at a temperature ramp-up rate of 10° C./min, a gradual drop in the weight of diphenylmethane diisocyanate can be observed from about 150° C. On the other hand, in a resin sample in which the reaction between the thermoplastic polyurethane material and the isocyanate mixture has been carried out to completion, a weight drop from about 150° C. is not observed, but a weight drop from about 230 to 240° C. can be observed.

After the resin composition has been molded as described above, its properties as a golf ball cover can be further improved by carrying out annealing so as to induce the crosslinking reaction to proceed further. "Annealing," as used herein, refers to aging the cover in a fixed environment for a fixed length of time.

In addition to the above resin components, various optional additives may be included in the cover material in the present invention. Such additives include, for example, pigments, dispersants, antioxidants, ultraviolet absorbers, ultraviolet stabilizers, parting agents, plasticizers, and inorganic fillers (e.g., zinc oxide, barium sulfate, titanium dioxide, tungsten).

When such additives are included, the amount of the additives is suitably selected from a range within which the objects of the invention are achievable, although it is preferable for such additives to be included in an amount, per 100 parts by weight of the thermoplastic polyurethane serving as an essential component of the invention, of preferably at least 0.1 part by weight, and more preferably at least 0.5 part by weight, but preferably not more than 10 parts by weight, and more preferably not more than 5 parts by weight.

Molding of the cover using the thermoplastic polyurethane of the invention may be carried out by using an injection-molding machine to mold the cover over the intermediate layer which encases the core. Molding is carried out at a molding temperature of generally from 150 to 250° C.

Next, the cover of the inventive golf ball has a thickness which, while not subject to any particular limitation, is preferably at least 0.5 mm, more preferably at least 0.7 mm, even more preferably at least 0.9 mm, and most preferably at least 1 mm, but preferably not more than 2 mm, more preferably not more than 1.8 mm, even more preferably not more than 1.6 mm, and most preferably not more than 1.4 mm. If the cover is thinner than the above range, the durability may worsen and cracking tends to arise, or the scuff resistance may worsen. On the other hand, if the cover is thicker than the above range, the feel on impact may worsen or an increase in distance may not be achieved.

The cover material in the invention has a Shore D hardness which, while not subject to any particular limitation, is preferably at least 47, more preferably at least 49, even more preferably at least 51, and most preferably at least 53, but preferably not more than 61, more preferably not more than 59, and most preferably not more than 57. At a low shore D hardness, the distance decreases. Conversely, if the shore D hardness is too high, the ball has a hard feel on impact.

The cover hardness is higher than the intermediate layer hardness, the Shore D hardness difference therebetween being preferably at least 1, more preferably at least 3, even

more preferably at least 5, and most preferably at least 7, but preferably not more than 15, more preferably not more than 13, even more preferably not more than 12, and most preferably not more than 11. Outside of the above hardness difference range, the durability to cracking may worsen or the feel on impact may worsen.

To achieve an excellent durability to cracking and an excellent flight performance, it is desirable for the cover and the intermediate layer to have a combined thickness of preferably at-least 2 mm, more preferably at least 2.3 mm, even more preferably at least 2.6 mm, and most preferably at least 2.9 mm, but preferably not more than 4 mm, more preferably not more than 3.7 mm, and even more preferably not more than 3.4 mm.

The golf ball diameter should accord with golf ball standards, and is preferably not less than 42.67 mm.

In the above range in the golf ball diameter, the deflection of the ball as a whole when compressed under a final load of 130 kgf from an initial load of 10 kgf (which deflection is also called the "product hardness") is preferably at least 2.4 mm, more preferably at least 2.6 mm, even more preferably at least 2.8 mm, and most preferably at least 3.0 mm, but preferably not more than 5.0 mm, more preferably not more than 4.5 mm, even more preferably not more than 4.0 mm, and most preferably not more than 3.8 mm.

In the present invention, the golf ball has an initial velocity of preferably at least 76.8 m/s, more preferably at least 77.0 m/s, and even more preferably at least 77.2 m/s, but preferably not more than 77.7 m/s, more preferably not more than 77.6 m/s, and even more preferably not more than 77.5 m/s. The initial velocity of the golf ball, which is defined in the same way as the definition of the initial velocities of the core and the sphere I, is a value obtained by the same method of measurement as the method described in the subsequent examples. That is, it is a value measured using an initial velocity measuring apparatus of the same type as a USGA drum rotation-type initial velocity instrument approved by the R&A.

To increase the aerodynamic performance and extend the distance traveled by the ball, the number of dimples formed on the ball surface is preferably at least 250, more preferably at least 270, even more preferably at least 290, and most preferably at least 300, but preferably not more than 400, more preferably not more than 380, even more preferably not more than 360, and most preferably not more than 340.

The sum of the dimple trajectory volumes VT (total dimple trajectory volume TTV) obtained by multiplying the volume V of each dimple by the square root of the dimple diameter  $D_i$  is preferably at least 640, more preferably at least 645, even more preferably at least 650, and most preferably at least 655, but preferably not more than 800, more preferably not more than 770, even more preferably not more than 740, and most preferably not more than 710. In the present invention, TTV is the sum of the VT ( $=V \times D_i^{0.5}$ ) for each dimple. Here, the dimple volume V, although not shown in the diagrams, is the volume of the recessed region circumscribed by the edge of a dimple. The approximate trajectory height at high head speeds, particularly at head speeds of about 45 m/s to about 55 m/s, can be determined from this TTV value. Generally, the angle of elevation is large at a small TTV value, and is small at a large TTV value. At too small a TTV value, the trajectory will be too high, resulting in an insufficient run and thereby shortening the total distance. On the other hand, at too large a TTV value, the trajectory will be too low, resulting in an insufficient carry and likewise shortening the distance. Moreover, outside the TTV range of the invention, the ball will

have a large variability in the carry, lowering the stability of the ball performance in all such cases.

In the present invention, the respective initial velocities (m/s) of the core, the sphere I composed of the core encased by the intermediate layer, and the golf ball must satisfy Formula A:  $(\text{initial velocity of core} - \text{initial velocity of sphere I})^2 + (\text{initial velocity of sphere I} - \text{initial velocity of golf ball})^2 < 0.40$ . By satisfying this formula and satisfying the subsequently described formula B, it is possible to achieve a golf ball which has an excellent feel on impact, durability to cracking and scuff resistance and which also has an excellent distance due to a reduced spin rate on full shots. The upper limit in the value expressed by the above formula (initial velocity of core - initial velocity of sphere I)<sup>2</sup> + (initial velocity of sphere I - initial velocity of golf ball)<sup>2</sup> is preferably not more than 0.35, more preferably not more than 0.30, and even more preferably not more than 0.25.

Also, in the present invention, the respective deflections (mm) of the core, the sphere I composed of the core encased by the intermediate layer, and the golf ball, when compressed under a final load of 130 kg from an initial load of 10 kgf, must satisfy Formula B:  $0.30 < (\text{deflection of core} - \text{deflection of sphere I})^2 + (\text{deflection of sphere I} - \text{deflection of golf ball})^2 < 0.70$ . The reason is the same as that given above in connection with Formula A. The lower limit in the value expressed by the above formula (deflection of core - deflection of sphere I)<sup>2</sup> + (deflection of sphere I - deflection of golf ball)<sup>2</sup> is preferably at least 0.35, more preferably at least 0.40, and even more preferably at least 0.45, and the upper limit is preferably not more than 0.65, more preferably not more than 0.60, and even more preferably not more than 0.55.

In addition, it is preferable for the thicknesses and material hardnesses of the intermediate layer and the cover to satisfy formula C below.

$$0 < [\text{material hardness (Shore D)} \times \text{intermediate layer thickness (mm)}] - [\text{material hardness (Shore D)} \times \text{cover thickness (mm)}] < 40$$

Formula C

In the above formula, the value expressed as [material hardness (Shore D) of intermediate layer × intermediate layer thickness (mm)] - [material hardness (Shore D) of cover × cover thickness (mm)] is more preferably at least 5, even more preferably at least 10, and most preferably at least 15, but more preferably not more than 35, even more preferably not more than 30, and most preferably not more than 25. If the above value is too much larger than the above range, the feel and durability of the ball may worsen. On the other hand, if the above value is too much smaller than the above, the distance traveled by the ball may decrease.

In addition, it is preferable for the thicknesses of the intermediate layer and the cover to satisfy formula D below.

$$1.2 < \text{intermediate layer thickness} / \text{cover thickness} < 1.7$$

Formula D:

The above intermediate layer thickness/cover thickness value is more preferably at least 1.3, and even more preferably at least 1.4, but more preferably not more than 1.7, even more preferably not more than 1.6, and most preferably not more than 1.5. If this value is too much larger than the above range, the distance traveled by the ball may not increase. On the other hand, if the above value is too much smaller than the above range, the feel and durability of the ball may worsen and the distance may decrease.

As explained above, the multi-piece solid golf ball of the invention, by minimizing the differences in initial velocity between the respective layers and optimizing at a small value the differences in deflection under specific loading between the respective layers, can be imparted with a good feel on

impact and an excellent spin performance on approach shots, in addition to which a lower spin rate can be achieved on full shots, enabling the distance of the ball to be improved and also resulting in an excellent scuff resistance and durability.

## EXAMPLES

The following Examples and Comparative Examples are provided by way of illustration and not by way of limitation.

## Examples 1 to 8, Comparative Examples 1 to 5

Solid cores were fabricated by preparing core compositions in the respective formulations No. 1 to No. 9 shown in Table 1, then molding and vulcanizing under the vulcanization conditions shown in the tables.

TABLE 1

|                                    | No. 1 | No. 2 | No. 3 | No. 4 | No. 5 | No. 6 | No. 7 | No. 8 | No. 9 |
|------------------------------------|-------|-------|-------|-------|-------|-------|-------|-------|-------|
| Butadiene rubber                   | 100   | 100   | 100   | 100   | 100   | 100   | 100   | 100   | 100   |
| Zinc acrylate                      | 27.0  | 25.0  | 29.5  | 28.5  | 27.5  | 27.5  | 31.0  | 24.5  | 24.5  |
| Peroxide (1)                       | 0.3   | 0.3   | 0.3   | 0.3   | 0.3   | 0.3   | 0.3   | 0.3   | 0.3   |
| Peroxide (2)                       | 0.3   | 0.3   | 0.3   | 0.3   | 0.3   | 0.3   | 0.3   | 0.3   | 0.3   |
| Zinc oxide                         | 5     | 5     | 5     | 5     | 5     | 5     | 5     | 5     | 5     |
| Barium sulfate                     | 31.8  | 32.5  | 31.0  | 30.8  | 31.5  | 19.4  | 30.5  | 32.4  | 32.8  |
| Antioxidant                        | 0.1   | 0.1   | 0.1   | 0.1   | 0.1   | 0.1   | 0.1   | 0.1   | 0.1   |
| Zinc salt of pentachlorothiophenol | 0.3   | 0.5   | 0.1   | 1     | 0.5   | 0.3   | 0     | 1     | 0.3   |
| Zinc stearate                      | 5     | 5     | 5     | 5     | 5     | 0     | 5     | 5     | 5     |
| Specific gravity                   | 1.23  | 1.23  | 1.23  | 1.23  | 1.23  | 1.174 | 1.23  | 1.23  | 1.217 |
| Deflection (mm)                    | 4.1   | 4.6   | 3.5   | 3.9   | 4.1   | 3.7   | 3.2   | 5     | 4.6   |

Numerical values for the formulations in the table indicate parts by weight.

Butadiene rubber: "BR01"; available from JSR Corporation.

Zinc acrylate: Available from Nihon Jyoryu Kogyo Co., Ltd.

Peroxide (1): "Percumyl D"; available from NOF Corporation.

Peroxide (2): "Perhexa C-40"; available from NOF Corporation.

Zinc oxide: Available from Sakai Chemical Industry Co., Ltd.

Barium sulfate: "Chinkosei Ryusan Barium 100"; available from Sakai Chemical Industry Co., Ltd.

Antioxidant: "Nocrac NS-6"; available from Ouchi Shinko Chemical Industry Co., Ltd.

Zinc stearate: "Zinc Stearate G"; available from NOF Corporation.

Next, an intermediate layer and a cover were formed over the solid core by injection molding, in this order, the respective resin materials shown in Table 2. The dimple arrangement used in each case was the same: Dimple type I (336 dimples in the pattern shown in FIG. 2).

TABLE 2

|                         | A    | B    | C    | D   | E   | F   | G   | H |
|-------------------------|------|------|------|-----|-----|-----|-----|---|
| Himilan 1557            |      |      | 42.5 | 40  | 52  |     | 30  |   |
| Himilan 1601            |      |      | 42.5 |     | 48  |     |     |   |
| Himilan 1605            | 68.5 |      |      |     |     |     | 50  |   |
| Himilan 1706            |      |      |      |     |     |     | 25  |   |
| Himilan 1855            |      |      | 10   |     |     | 20  |     |   |
| Himilan AM7331          |      |      | 50   |     |     | 50  |     |   |
| Himilan AM7329          |      |      |      |     |     |     | 25  |   |
| Pandex T8295            |      |      |      | 100 |     |     |     |   |
| Nucrel AN4318           |      | 15   |      |     |     |     |     |   |
| Nucrel AN4319           | 84   |      |      |     |     |     |     |   |
| Nucrel 1560             | 1    |      |      |     |     |     |     |   |
| Dynaron 6100P           | 15   | 31.5 |      |     |     |     |     |   |
| Polyisocyanate compound |      |      |      |     | 9   |     |     |   |
| Thermoplastic elastomer |      |      |      |     | 15  |     |     |   |
| Titanium oxide          |      | 4.8  | 2.2  | 3   | 3.5 | 2.2 | 2.8 |   |
| Polyethylene wax        |      |      |      |     | 1.5 |     | 1   |   |
| Calcium hydroxide       | 2.3  |      |      |     |     |     |     |   |
| Polytail H              | 2    |      |      |     |     |     |     |   |
| Behenic acid            | 18   |      |      |     |     |     |     |   |

TABLE 2-continued

|                    | A  | B | C | D | E | F   | G | H   |
|--------------------|----|---|---|---|---|-----|---|-----|
| Magnesium oxide    | 1  |   |   |   |   |     |   |     |
| Magnesium stearate | 59 |   |   |   | 1 | 0.6 | 1 | 1.7 |

Numerical values for the formulations in the table indicate parts by weight.

Himilan: Ionomer resins available from DuPont-Mitsui Polychemicals Co., Ltd.

Pandex T8295: MDI-PTMG type thermoplastic polyurethane available from DIC Bayer Polymer.

Nucrel 1560: Copolymer available from DuPont-Mitsui Polychemicals Co., Ltd.

Dynaron 6100P: Thermoplastic block copolymer having a crystalline polyolefin block and a polyethylene/butylene copolymer, available from JSR Corporation

Polyisocyanate compound: 4,4-Diphenylmethane diisocyanate

Thermoplastic elastomer: "Hytrel 4001"; available from DuPont-Toray Co., Ltd.

Titanium oxide: "Tipaque R550"; available from Ishihara Sangyo Kaisha, Ltd.

TABLE 2-continued

|                                                                                                     | A | B | C | D | E | F | G | H |
|-----------------------------------------------------------------------------------------------------|---|---|---|---|---|---|---|---|
| Polyethylene wax: "Sanwax 161P"; available from Sanyo Chemical Industries, Ltd.                     |   |   |   |   |   |   |   |   |
| Calcium hydroxide: "CLS-B"; available from Shiraishi Calcium Kaisha, Ltd.                           |   |   |   |   |   |   |   |   |
| Polytail H: A low-molecular-weight polyolefin polyol available from Mitsubishi Chemical Corporation |   |   |   |   |   |   |   |   |
| Behenic acid: Available from NOF Corporation under the trade name "NAA-222S"                        |   |   |   |   |   |   |   |   |
| Magnesium oxide: "Kiyowamag MF150"; available from Kyowa Chemical Industry                          |   |   |   |   |   |   |   |   |
| Magnesium stearate: "Magnesium Stearate G"; available from NOF Corporation                          |   |   |   |   |   |   |   |   |

The following ball properties were measured in the resulting golf balls. In addition, flight tests were carried out by the method described below, and the spin rate on approach shots, feel on impact, durability to cracking and scuff resistance were evaluated. The results are given in Table 3 (examples of the invention) and Table 4 (comparative examples).

Deflection of Core, Intermediate Layer and Finished Product

The test sphere was placed on a hard plate and the deflection (mm) of the sphere when compressed under a final load of 1,275 N (130 kgf) from an initial load of 98 N (10 kgf) was measured.

## Core Surface Hardness

The Shore D hardness at the core surface was measured.

Measurements of the surface hardness were carried out at two places each on N=5 specimens. The Shore D hardnesses

are values measured in accordance with ASTM D-2240 after temperature conditioning at 23° C.

## Material Hardnesses of Intermediate Layer and Cover

The Shore D hardnesses were measured in accordance with the criteria of ASTM D-2240.

## Initial Velocities of Core, Intermediate Layer-Covered Sphere I, and Golf Ball

The initial velocity was measured using an initial velocity measuring apparatus of the same type as the USGA drum rotation-type initial velocity instrument approved by the R&A. The test spheres (core, intermediate layer-enclosed Sphere I and golf ball) were held isothermally at a temperature of  $23 \pm 1^\circ \text{ C.}$  for at least 3 hours, then tested in a room temperature ( $23 \pm 2^\circ \text{ C.}$ ) chamber. The balls were hit using a 250-pound (113.4 kg) head (striking mass) at an impact velocity of 143.8 ft/s (43.83 m/s). A dozen balls were each hit four times. The time taken for the test spheres to traverse a distance of 6.28 ft (1.91 m) was measured and used to compute the initial velocity. This cycle was carried out over a period of about 15 minutes.

### Distance with W#1

Each ball was struck ten times at a head speed (HS) of 45 m/s with the Tour Stage X-Drive (loft angle, 10.5°) driver (manufactured by Bridgestone Sports Co., Ltd.) mounted on a golf swing robot, and the spin rate (rpm) and total distance (m) were measured.

### (iii) Were measured:

#### Spin on Approach Shots

The spin rate (rpm) of the ball when struck at a head speed (HS) of 20 m/s with the Tour Stage X-Wedge (loft angle, 58°)

sand wedge (SW) (manufactured by Bridgestone Sports Co., Ltd.) mounted on a golf swing robot was measured.

### Durability to Cracking

The ball was repeatedly fired against a steel plate wall at an incident velocity of 43 m/s, and the number of shots taken until the ball cracked was determined. The average value for N=5 specimens was determined, and the durability was rated according to the following criteria.

Good: 200 or more shots

NG: less than 200 shots

Fee1

Three top amateur golfers rated the feel of the balls according to the following criteria when struck with a driver (W#1) at a head speed (HS) of 40 to 45 m/s.

Good: Good feel

Fair: Somewhat hard or somewhat soft

NG: Too hard or too soft

### Scuff Resistance

The golf balls were hit at a head speed of 40 m/s using a pitching wedge mounted on a swing robot, after which the condition of the ball's surface was visually rated according to the following scale.

Good: Can be used again

NG: No longer fit for use

TABLE 3

TABLE 4

|                    |                                                                           | Comparative Example |       |       |       |       |
|--------------------|---------------------------------------------------------------------------|---------------------|-------|-------|-------|-------|
|                    |                                                                           | 1                   | 2     | 3     | 4     | 5     |
| Core               | Formulation                                                               | No. 7               | No. 8 | No. 5 | No. 1 | No. 9 |
|                    | Diameter (mm)                                                             | 36.1                | 36.1  | 36.1  | 36.1  | 36.6  |
|                    | Deflection (10-130 kg) (mm)                                               | 3.2                 | 5.0   | 4.1   | 4.1   | 4.7   |
|                    | Surface hardness (Shore D)                                                | 49                  | 40    | 43    | 43    | 41    |
|                    | Initial velocity (m/s)                                                    | 77.7                | 77.5  | 77.8  | 77.4  | 77.3  |
| Intermediate layer | Material                                                                  | A                   | A     | A     | A     | A     |
|                    | Hardness (Shore D)                                                        | 48                  | 48    | 48    | 48    | 48    |
|                    | Diameter (mm)                                                             | 40.0                | 40.0  | 40.0  | 40.0  | 39.7  |
|                    | Thickness (mm)                                                            | 1.95                | 1.95  | 1.95  | 1.95  | 1.55  |
|                    | Deflection (10-130 kg) (mm)                                               | 2.9                 | 4.3   | 3.5   | 3.5   | 4.0   |
| Cover              | Initial velocity (m/s)                                                    | 77.5                | 77.3  | 77.7  | 77.4  | 77.2  |
|                    | Material                                                                  | C                   | E     | G     | H     | E     |
|                    | Hardness (Shore D)                                                        | 57                  | 60    | 53    | 63    | 60    |
|                    | Thickness (mm)                                                            | 1.35                | 1.35  | 1.35  | 1.35  | 1.5   |
|                    | Ball                                                                      | 42.7                | 42.7  | 42.7  | 42.7  | 42.7  |
| Ball               | Diameter (mm)                                                             | 45.4                | 45.4  | 45.4  | 45.4  | 45.4  |
|                    | Weight (g)                                                                | 2.50                | 3.70  | 3.30  | 2.90  | 3.50  |
|                    | Deflection (10-130 kg) (mm)                                               | 77.4                | 77.2  | 77.0  | 77.4  | 77.2  |
|                    | Initial velocity (m/s)                                                    | 0.05                | 0.05  | 0.50  | 0.00  | 0.01  |
|                    | Formula A                                                                 | 0.25                | 0.85  | 0.40  | 0.72  | 0.74  |
| W#1                | Formula C                                                                 | 16.7                | 12.6  | 22.1  | 8.5   | -15.6 |
|                    | Formula D                                                                 | 1.44                | 1.44  | 1.44  | 1.44  | 1.03  |
|                    | Hardness difference between intermediate layer and core surface (Shore D) | -1                  | 8     | 5     | 5     | 7     |
|                    | Spin rate (rpm)                                                           | 2820                | 2410  | 2740  | 2580  | 2460  |
|                    | Total distance (m)                                                        | 237.9               | 233.6 | 233.9 | 237.6 | 235.4 |
| SW                 | Spin rate (rpm)                                                           | 5840                | 5090  | 5900  | 4890  | 4960  |
|                    | Durability to cracking                                                    | good                | NG    | good  | good  | NG    |
|                    | Feel                                                                      | NG                  | fair  | good  | NG    | fair  |
|                    | Scuff resistance                                                          | NG                  | good  | NG    | good  | good  |

In Comparative Example 1, the formula B value was too small. As a result, the ball had a hard feel and a poor scuff resistance.

In Comparative Example 2, the formula B value was too large. As a result, the ball did not achieve a sufficient distance on shots with a W#1, and had a poor durability to cracking.

In Comparative Example 3, the formula A value was too large. As a result, the ball did not achieve a sufficient distance on shots with a W#1, and had a poor scuff resistance.

In Comparative Example 4, the formula B value was too large. As a result, the ball had a poor receptivity to spin on approach shots and also had a hard feel.

In Comparative Example 5, the formula B value was too large. As a result, the ball had a poor receptivity to spin on approach shots and also had a poor durability to cracking.

The invention claimed is:

1. A multi-piece solid golf ball comprising a solid core, a cover, at least one intermediate layer interposed therebetween, and a plurality of dimples on a surface of the ball, wherein the respective initial velocities (m/s) of the core, a sphere I composed of the core encased by the intermediate layer, and the golf ball, as measured by a method set forth in the Rules of Golf using an initial velocity measuring apparatus of the same type as a USGA drum rotation-type initial velocity instrument, satisfy formula A below, the respective deflections (mm) of the core, the sphere I composed of the core encased by the intermediate layer, and the golf ball, when compressed under a final load of 130 kgf from an initial load of 10 kgf, satisfy formula B below, and a relationship between the thickness of the intermediate layer and that of the cover layer satisfies formula D below:

$$\text{initial velocity of core-initial velocity of sphere I}^2 + \text{initial velocity of sphere I-initial velocity of golf ball}^2 < 0.40;$$

Formula A:

$$0.30 < (\text{deflection of core-deflection of sphere I})^2 + (\text{deflection of sphere I-deflection of golf ball})^2 < 0.70.$$

Formula B:

$$1.2 < \text{intermediate layer thickness/cover thickness} < 1.7;$$

Formula D:

wherein the cover has a material hardness that is higher than a material hardness of the intermediate layer material hardness, and which satisfies formula C below:

$$0 < [\text{material hardness (Shore D) of intermediate layer} \times \text{intermediate layer thickness (mm)}] - [\text{material hardness (Shore D) of cover} \times \text{cover thickness (mm)}] < 40.$$

Formula C

2. The multi-piece solid golf ball of claim 1, wherein the intermediate layer is composed primarily of a material obtained by mixing under applied heat:

100 parts by weight of a resin component of

(a) from 95 to 50 wt % of an olefin-unsaturated carboxylic acid-unsaturated carboxylic acid ester random terpolymer and/or a metal salt thereof,

(b) from 0 to 10 wt % of an olefin-unsaturated carboxylic acid random copolymer and/or a metal salt thereof, and

(c) from 5 to 50 wt % of a thermoplastic block copolymer having a crystalline polyolefin block and a polyethylene/butylene random copolymer,

with

(d) from 5 to 100 parts by weight of a fatty acid or fatty acid derivative having a molecular weight of from 280 to 1500, and

(e) from 0.1 to 10 parts by weight of a basic inorganic metal compound capable of neutralizing acid groups within components (a), (b) and (d);

and the intermediate layer has a Shore D hardness difference with a surface of the solid core of within  $\pm 10$ .

**29**

3. The multi-piece solid golf ball of claim 1, wherein the intermediate layer is composed primarily of a material obtained by mixing under applied heat:
- 100 parts by weight of a resin component of
- (a) from 0 to 20 wt % of an olefin-unsaturated carboxylic acid-unsaturated carboxylic acid ester random terpolymer and/or a metal salt thereof, 5
- (b) from 95 to 50 wt % of an olefin-unsaturated carboxylic acid random copolymer and/or a metal salt thereof, and
- (c) from 5 to 50 wt % of a thermoplastic block copolymer having a crystalline polyolefin block and a polyethylene/butylene random copolymer, 10

**30**

- with
- (d) from 5 to 100 parts by weight of a fatty acid or fatty acid derivative having a molecular weight of from 280 to 1500, and
- (e) from 0.1 to 10 parts by weight of a basic inorganic metal compound capable of neutralizing acid groups within components (a), (b) and (d);
- and the intermediate layer has a Shore D hardness difference with a surface of the solid core of within  $\pm 10$ .

\* \* \* \* \*